

## UNITED STATES PATENT OFFICE

2,658,871

## LUBRICATING COMPOSITION

Paul V. Smith, Jr., Westfield, and James B. McPherson, Jr., Roselle, N. J., assignors to Standard Oil Development Company, a corporation of Delaware

No Drawing. Application September 3, 1949,  
Serial No. 114,066

4 Claims. (Cl. 252—49.8)

1

This invention relates to lubricants having a high degree of oiliness, and more particularly to a lubricating composition which contains combined therein an ester of phosphoric acid to impart oiliness and film strength thereto. It is especially directed toward a lubricating composition which contains an oxo alcohol ester of a phosphoric acid.

In the lubricant art, considerable progress has been realized in recent years in the production of lubricants characterized by one or more specific properties and adapted for particular uses. In the main, this progress can be attributed to two developments: the first, new refining procedures, and the second, addition agents capable of imparting particular properties to available lubricants. Thus, viscosity index improvers and pour depressants are added to automotive lubricants to render the lubricants more adaptable to wide changes in temperature conditions, while other agents are added to improve the load carrying properties of a lubricant which is to be employed, for example, under extreme pressure conditions.

Certain machine elements, such as the hypoid gears commercially used in automotive vehicles, may be subjected at times to extremely heavy pressures of the order of hundreds of thousands of pounds per square inch. Under these conditions, if the film of lubricating oil separating the opposed elements fails, as it is likely to do under such pressure, the surfaces contact each other directly with resultant seizure or excessive wear and early failure. To combat this deficiency in lubricating oils, a group of compounds known as "extreme pressure additives" has been developed. Extreme pressure additives contain active sulfur, phosphorus, chlorine or the like which react with the metal surfaces at the high temperatures generated by friction when machine elements operate at extremely high pressures. The presence of reactive chlorine and the like in a lubricating oil is detrimental to some extent in that it subjects the metallic elements lubricated to corrosive action. There is, accordingly, no advantage but, on the contrary, severe disadvantage to using extreme pressure lubricants where they are not essential.

A wide intermediate area lies between lubrication requirements; between those (1) requiring an extreme pressure lubricant and (2) those that may be met satisfactorily with straight run mineral oils. In this area an oil is required having a high film strength but which does not require

2

extreme pressure action. It is toward the requirements of this intermediate area that the lubricating composition of this invention is directed.

It has been known in the lubricating art that the esters of phosphoric acid make very good extreme pressure additives for lubricating oils. For example, Benning in U. S. Patent 2,167,867 teaches that an oil composition containing the alkyl or aryl esters of phosphoric acid is a good lubricant for cadmium-silver bearings. In U. S. Patent 2,252,133 Morway et al. teach that a valuable metal fabricating oil may be made by slightly sulfurizing an oil and incorporating therein an aliphatic or an aryl ester of phosphoric acid. Downing et al., in U. S. Patents 2,285,853-4 teach the improvement of lubricants by the addition of aryl or aliphatic esters of phosphoric acid. Knutson et al. in U. S. Patent 2,340,331 teach the combination of various organic derivatives of inorganic oxy-acids with a lubricant to improve the extreme pressure properties thereof.

It has recently been discovered that the esters of phosphoric acid made from oxo alcohols have excellent potency as oiliness or film-strengthening agents for lubricating oils. These oxo alcohol esters of phosphoric acid are made by treating the oxo alcohol with phosphorus oxychloride under suitable conditions. The various oxo alcohols are made by the so-called "oxo synthesis" process. This process may be described as the catalytic reaction of mono-olefins with carbon monoxide and hydrogen at a temperature of about 300 to 350° F. and under a pressure of about 3000 pounds per square inch to form an aldehyde, and the subsequent hydrogenation of the aldehyde to form a primary alcohol. The process was first developed in Germany and was first described in this country in U. S. Patent 2,327,066, issued to Roelen in 1943. Depending upon the starting olefin, various alcohols may be synthesized by this process. For example, a C<sub>7</sub> fraction isolated from the product of the polymerization of propylene or a mixture of C<sub>3</sub> and C<sub>4</sub> olefins, may be subjected to the oxo process and the resulting C<sub>8</sub> oxo alcohol will be found to include a number of isomers having, on the average, two alkyl side groups along a carbon chain 4 to 6 carbon atoms in length.

Heretofore, it has been proposed to separate out a pure oxo alcohol from the crude product of the oxo process to form the phosphoric acid ester to combine with a lubricating oil. This procedure necessitates an expensive and time

consuming fractionating process which makes it undesirable from an economic standpoint.

It has now been found that when the crude oxo product is used as an esterifying agent, a more effective additive is formed than when the purified oxo alcohol is used. Thus a double advantage is gained; a more effective agent is obtained and an expensive fractionating process is eliminated.

Accordingly, this invention has as its primary object the formation of a superior lubricant by incorporating into a mineral base lubricating oil the desired amount of an ester of phosphoric acid obtained by reacting phosphorus oxychloride with the crude product of an oxo reaction.

Although in its preferred embodiment the invention contemplates the use of a crude C<sub>8</sub> oxo alcohol, it is to be understood, of course, that any of the oxo alcohols in their crude state may be used without departing from the concept of the invention. For example, a crude C<sub>9</sub> cut, a crude C<sub>11</sub>-C<sub>12</sub> fraction, a crude C<sub>12</sub>-<sub>13</sub> fraction, or a crude C<sub>13</sub>-<sub>44</sub> cut of alcohols made by the oxo process may be used.

The process by which the crude phosphate is prepared is as follows:

Crude C<sub>8</sub> oxo alcohol, containing an amine such as pyridine, dimethyl amine, diethyl amine, etc., is treated with POCl<sub>3</sub>, at a temperature ranging from about -10° to about +10° C. The amine is present to tie up the released hydrochloric acid and can be regenerated and used again. The mixture is refluxed several hours, diluted with water, and the organic layer washed with water, salt solution, or dilute sodium carbonate until neutral. The mixture is then heated to 180 to 190° C. under 5 to 6 mm. vacuum, the volatile constituents being taken overhead. The material remaining in the flask is used directly as the crude ester. This crude ester was fractionally distilled, taking overhead at 198° C. and at 4 mm. pressure a pure phosphate fraction for comparative use.

An analysis of the crude C<sub>8</sub> oxo phosphate is given below:

|                  |                                                                                                         |
|------------------|---------------------------------------------------------------------------------------------------------|
| Hydroxy          | 0.011 centiequivalent/gm.                                                                               |
| Acid             | 0.012 centiequivalent/gm.<br>(this corresponds to 3.8<br>wt. percent calculated<br>as the diphosphate). |
| Acetal           | 0.006 centiequivalent/gm.                                                                               |
| Carbonyl         | 0.004 centiequivalent/gm.                                                                               |
| H <sub>2</sub> O | 0.0 centiequivalent/gm.                                                                                 |
| Bromine No.      | 0.18 centiequivalent/gm.                                                                                |
| Ash              | 5.21 centiequivalent/gm.                                                                                |

All of these impurities are higher boiling than the pure C<sub>8</sub> oxo phosphate.

Various concentrations of the crude ester of phosphoric acid in a solvent extracted coastal distillate having a viscosity at 210° F. of 45 S. U. S. were prepared and tested in the 4-ball testing machine. This machine is designed to test lubricants under conditions of pressure to determine their film strength characteristics. The machine is so constructed that one steel ball contacts and rotates upon three stationary steel balls of identical physical properties. The lubricant being tested is placed upon the contacting surfaces and the desired load is applied upon the single rotating ball. Wear scars appearing upon the three stationary balls are measured and averaged, their diameters being a function of the film strength of the lubricant undergoing the test. The results of the tests on materials pre-

pared in accordance with the concept of this invention are given in Table I below:

TABLE I  
4-ball test machine data

| Additive percent in<br>Oil A <sup>1</sup> | Wear Scar Diameter mm. (30 min. test<br>at 20 Kg. Load) |                               |               |                |
|-------------------------------------------|---------------------------------------------------------|-------------------------------|---------------|----------------|
|                                           | Comm'l<br>Agt. A <sup>2</sup>                           | Comm'l<br>Agt. B <sup>3</sup> | Pure<br>Ester | Crude<br>Ester |
| 0.0                                       |                                                         | 0.58<br>(not run)             | 0.37          | 0.26           |
| 0.5                                       | 0.30                                                    | do                            | 0.35          | 0.26           |
| 1.0                                       | 0.28                                                    | 0.50                          | 0.37          | 0.25           |
| 2.0                                       | 0.28                                                    |                               |               |                |

<sup>1</sup> Solvent extracted coastal distillate having a viscosity at 210° F. of 45 S. U. S.

<sup>2</sup> Tricresyl phosphate type.

<sup>3</sup> Fatty acid ester type.

It will be noted from a study of Table I above that outstanding results are obtained when using the product of this invention, the wear scars showing a decided improvement over both the pure ester and the commercial additives. These results are particularly outstanding since the Hertz inelastic compression of the balls of the testing machine is about 0.24 mm. under a 20 kg. load. It can readily be seen that with the additive of this invention the wear is practically eliminated.

Although the commercial additive A shows wear scars only slightly greater than those of the crude ester, a very favorable economic advantage exists in the product of this invention, and since an expensive fractional distillation procedure is eliminated the products prepared according to this invention are prepared at a great reduction in cost over the pure ester.

Although the additive material of this invention is preferably employed in a mineral base lubricating oil, it is operable to improve the oiliness or film strength of any lubricating oil, either natural or synthetic. It may be combined with the base stock in amounts varying from 0.5 to 10%, 0.5 to 3.0% ordinarily sufficing to obtain the desired improvement.

The crude C<sub>8</sub> oxo phosphate is also very useful as an additive for spindle oils in which service its excellent film strength imparting characteristic is particularly advantageous. A typical spindle oil was prepared using the crude C<sub>8</sub> oxo phosphate, pure C<sub>8</sub> oxo phosphate and the commercial additive A, described in Table I, on the following formulation:

600 grams of a solvent extracted Rhodessa distillate having a viscosity of 210° F. of 41 S. U. S.  
0.1% of a commercial oxidation inhibitor.  
0.075% of a commercial detergent inhibitor.  
1.0% of oiliness agent.

These prepared spindle oils were subjected to the Staeger life test, well known to the lubricating art, which is designed to measure the oxidation of a lubricant under typical operating conditions. An oven maintained at a constant temperature of 110° C. is equipped with an aluminum shelf which is motor driven at from 5 to 6 revolutions per minute. The shelf contains holes to allow for free air circulation. Air, which is purified by being bubbled through an 8-10% solution of potassium hydroxide, an 8-10% solution of silver nitrate, and finally a concentrated solution of sulfuric acid, is blown through the oven at a rate of 1.5 to 2 cubic feet per hour. A 200 cubic centimeter sample of the oil to be tested is placed on the rotating shelf and a clean

standard size copper strip (40 x 70 x 1 mm.) is placed in the sample, the copper strip serving as a catalyst for oxidation. At various stages of the test period, samples of the test oil are removed and a neutralization number obtained by the ASTM D188-27T method, the acidity of the sample increasing in direct ratio to the amount of oxidation. The Staeger life of a lubricant is defined as being the number of hours in the test oven necessary to raise the neutralization number 0.20. The results of the Staeger life test on the above spindle oil formulation are given in Table II below:

TABLE II  
Staeger life test

| Time<br>(Hours) | Commercial<br>Additive A<br>(Neut. No.) | Oiliness Additive                                   |                                                      |
|-----------------|-----------------------------------------|-----------------------------------------------------|------------------------------------------------------|
|                 |                                         | Pure C <sub>8</sub> Oxo<br>Phosphate<br>(Neut. No.) | Crude C <sub>8</sub> Oxo<br>Phosphate<br>(Neut. No.) |
| 0.....          | 0.15.....                               | 0.20.....                                           | 0.14.....                                            |
| 215.....        | 0.24.....                               | (not run).....                                      | (not run).....                                       |
| 282.....        | 0.56.....                               | 0.30.....                                           | 0.27.....                                            |
| 330.....        | (not run).....                          | 0.70.....                                           | 0.38.....                                            |

Examination of the test data given above shows a Staeger Life on the spindle oil containing the product of this invention of slightly less than 320 hours. This compares very favorably with the value of less than 235 hours for the spindle oil containing the commercial additive A, or a life of approx. 290 hours for the spindle oil having the pure C<sub>8</sub> oxo phosphate incorporated therein.

To recapitulate briefly, the present invention comprises the discovery that a greatly improved film strengthening or oiliness agent for incorporation into mineral based lubricating oils to improve the film strength or oily characteristics thereof may be prepared by reacting the crude C<sub>8</sub> alcohol mixture resulting when polymers of propylene and butene are submitted to the oxo process with phosphoric oxychloride in the presence of an amine derivative followed by water 45 washing and stripping to 180 to 190° C. 5-6 mm. vacuum.

It is to be understood that the lubricating com-

position of this invention may include other additives for imparting desirable characteristics to lubricating oils, such as extreme pressure additives, corrosion inhibitors, anti-oxidants, viscosity index improvers, pour depressors and the like.

What is claimed is:

1. A lubricating composition which comprises a major amount of a mineral lubricating oil having combined therewith about 0.5 to 3.0% by weight of an ester of phosphoric acid, said ester being formed by reacting phosphorus oxychloride with the crude product obtained by subjecting a copolymer of propylene and butylene to the oxo process.
- 15 2. A lubricating composition which comprises a major amount of a mineral lubricating oil having combined therewith about 0.5 to 3.0% by weight of an ester of phosphoric acid, said ester being formed by reacting phosphorus oxychloride with the crude product obtained by subjecting a copolymer of propylene and butylene to the action of carbon monoxide and hydrogen in the presence of a cobalt catalyst at a temperature in the range of from 300 to 350° F. at a pressure of about 3000 pounds per square inch gauge and hydrogenating the aldehydes so formed.
- 20 3. A lubricating composition which comprises a major amount of a mineral base lubricating oil with about 0.5 to 10% by weight of a phosphoric acid ester of a crude C<sub>8</sub> oxo alcohol.
- 25 4. A lubricating composition which comprises a major amount of a mineral base lubricating oil with about 0.5 to 10% by weight of an unpurified product obtained by reacting phosphorus oxychloride with a crude C<sub>8</sub> oxo alcohol in the presence of pyridine.

PAUL V. SMITH, JR.  
JAMES B. MCPHERSON, JR.

References Cited in the file of this patent

UNITED STATES PATENTS

| Number    | Name           | Date          |
|-----------|----------------|---------------|
| 2,005,619 | Graves         | June 18, 1935 |
| 2,080,299 | Benning et al. | May 11, 1937  |
| 2,285,853 | Downing        | June 9, 1942  |
| 2,389,513 | Kemp           | Nov. 20, 1945 |